

July 5, 1938.

C. H. ALLEN

**2,122,394**

# THIN STOCK PROCESS AND APPARATUS FOR MAKING PAPER

Filed Oct. 6, 1936



INVENTOR  
Carlton H. Allen

## UNITED STATES PATENT OFFICE

2,122,394

THIN STOCK PROCESS AND APPARATUS  
FOR MAKING PAPER

Carlton H. Allen, Glens Falls, N. Y.

Application October 6, 1936, Serial No. 104,220

3 Claims. (Cl. 92—46)

This invention relates to the continuous process for making paper and the apparatus essential to this process.

The objects attained in the practice of the invention are a greater efficiency of the process, better quality paper and reduced cost of manufacture.

The improvements are particularly useful in the making of news and similar grades, but may be applied to advantage in the making of other grades where conditions are suitable. As will hereinafter become apparent, greater advantages are attained where the paper making pulp or pulps are produced at or near the paper mill. This is the usual situation wherever news print is manufactured, and this description is made with special reference to this paper.

According to the present most advanced practice as employed by the majority of manufacturers, solutions are made of each of the paper making ingredients which thereafter are flowed continuously through an apparatus for metering and proportioning each ingredient to form a composite paper stock, or a common stream of paper stock, and the consistency of the ground wood solution and the sulphite solution is held at a point somewhere between 2% and 4% by aid of thick stock consistency regulators, so-called. Some of the wood from which the paper is made, is ground mechanically, screened at a consistency of about 0.45% to remove the larger particles and dirt, and then thickened to a consistency of about 3.0% to form the ground wood solution. A smaller proportion of the wood is digested by the action of acid and heat, screened at a consistency of about 0.3% and then thickened to a consistency of about 2.5% to form the sulphite solution. The ground wood is thickened after screening by machines known as deckers or the operation may be accomplished by vacuum filters. Deckers permit the escape of nearly one third of the ground wood pulp which thereafter must be recovered and returned for re-screening and re-thickening. The recovery operation loads the screens making necessary additional screens, and loads the thickening machines making necessary additional deckers. The recovery operation is expensive in many ways, and in some mills the deckers have been replaced with vacuum filters in an effort to reduce the loss of pulp due to the thickening operation. About 14% of the pulp supplied to the filters escapes in the white water and as much as possible is recovered and returned to the system. Vacuum filters are ex-

pensive in first cost, expensive also in power required for their operation and in maintenance.

When ground wood pulp is deckered or filtered a separation of the fine from the coarser pulp takes place. The portion of the pulp retained on the filter surface is formed to a lumpy mass which must again be broken down to a solution before it is suitable to meter and run on the paper machine. The finer material which escapes to the white water system has a faculty for coating the inside of the pipe lines, forming slime which after a time becomes discolored, and upon loosening and travelling on through the system eventually causes black specks and slime spots in the finished paper with the result that the paper is poorer in quality and trouble is experienced in keeping the sheet from breaking on the paper machine.

Use of the herein described improvements in process eliminates most of the thickening operation and in some cases, all of the thickening operation which heretofore has been applied to a pulp. Either or both, the ground wood solution and the sulphite solution before metering are held at consistencies very like those required for screening. At these consistencies the mixing after metering is more thorough and efficient resulting in better formation of the paper making web. My process is more direct acting, giving less time and opportunity for troublesome lumps and slime to form in the pulp and in the pipe lines. The present necessities for separating the fine fibre and lignin of the ground wood pulp from the coarser and longer fibre of the same pulp and again reassembling the two classes of this pulp before metering are voided. Moreover, the cost of operating and maintaining deckers, filters and vacuum pumps is saved. Greater production of better quality paper at lowered cost is accomplished.

This invention is herein illustrated and described both as an improved process for making paper and as suitable apparatus in a preferred combination for practicing the invention, the accompanying drawing serving to illustrate the coordinated apparatus and improved process, the invention being defined in the appended claims within the limitations of the illustrations and description and also in the broader aspects contemplated in its general practice in the making of different kinds and grades of paper or the like.

In the drawing:

Fig. 1 is a view in elevation, partly in section and partly diagrammatic, illustrating an appa-

ratus in preferred form suitable for practicing the invention;

Fig. 2 is a view in elevation, partly in section and partly diagrammatic, illustrating an apparatus for controlling the consistency of a pulp solution at a value slightly lower than that required for screening a pulp-ingredient of the paper.

In the drawing, details of apparatus which would only serve to confuse the reader are omitted. The arrow-head lines indicate pipe lines and the arrow-heads show the direction of flow.

Referring now to Fig. 1: after grinding the ground wood pulp is pumped through line 1 to the screens 2, from where after screening, it drops through line 3 to vat 4 located on the main floor 5. At screening consistency, about 0.5%, the greater quantity of the screened pulp drops from vat 4 through line 6 to vat 7 located on the lower floor 8, the liquid level in which is controlled by 10 the float valve 9. Any quantity of the screened pulp not accepted in the vat 7 overflows the dam 10 of the vat 4 to the thickening machines 11, from which point thickened pulp of a consistency of about 3.0% drops through line 12 to the slush 15 pulp storage 13. From the slush storage 13, the thickened pulp flows to the vat 7 under control of the regulating valve 14. The mixture of the two streams of pulp in vat 7 is withdrawn continuously by a pump 15 and delivered to the 20 metering apparatus 16 on the main floor 5. A thin watery solution passes through pump 15 having a consistency somewhat higher than screening consistency, as for example a consistency of 0.65%. A small portion of the pulp passing through line 17 is diverted through line 18 to the thin stock indicator 19 from which point it is returned to vat 7 through line 20.

Instrument 19 is sensitive to changes in the consistency of the thin pulp passing through 25 pump 15 and it controls the operation of the power driven regulating valve 14, directing either a slow opening or closing movement of the valve 14 to maintain the consistency of the solution passing through pump 15 and the line 17 to the 30 metering apparatus 16 at a constant value of the magnitude desired.

Instrument 19 is fully illustrated and described in my application for patent, Serial No. 741,908, filed in the United States Patent Office August 50 23, 1934. In practice the instrument 19 has proven extremely sensitive to the consistency of a thin pulp solution and for the purpose here used it is especially well adapted.

The sulphite solution may be processed as described for the ground wood solution and flowed to the metering apparatus 16 through the line 21. Other ingredients required in the paper such as color and alum are also supplied to meter 16 through suitable lines (not shown).

60 A metering apparatus of the class required of meter 16 is fully shown and described in United States Patent No. 15,311 reissued to me and Edward J. Trimble March 21, 1922, and again in United States Patent No. 1,620,860 issued to me 65 March 15, 1927. Such metering apparatus is now well known and widely used by paper makers in the United States and in many foreign countries.

The meter 16 is understood to include one 70 meter for each ingredient of the paper stock. The meters are individually adjustable as to rate of metering to fix the proportion of ingredient to other ingredients. Further, all of the meters are interlocked mechanically in a way such that a 75 single adjustment of one master control may

change the rate of metering of each and all of the meters simultaneously to suit the capacity of the paper machine and without disturbing the proportion of any ingredient to the other ingredients.

From meter 16 a common stream of paper stock is discharged as a thin solution, for example 0.65% consistency, through line 22 to the paper machine fan pump 23 where it is joined to a stream of white water from the wire pit 24 flowing through line 25 to pump 23. Pump 23 mixes the paper stock and white water and discharges the mixture through line 26 and hand regulating valve 27 to the head box 28 and on to the paper machine wire 29. The rate at which white water 15 is drawn from pit 24 depends upon the setting of hand regulating valve 27, i. e. when this valve is given a greater opening more white water is drawn from pit 24 and when given a lesser opening less white water is drawn from the pit. Pit 24 is supplied only by water and stock which drains by gravity through wire 29 near the breast roll 30, thus forming a white water solution having a consistency of about 0.12% to 0.20%. Joining and mixing the stream of paper stock from 25 meter 16 with white water from pit 24 reduces the consistency of the paper stock flowing to wire 29 to a degree depending upon the rate of flow from pit 24 to pump 23, as for example to a consistency of 0.5%.

Paper stock as delivered to the wire of a paper machine is a thin solution, the consistency of which is different for different paper machines as determined by the length of wire, the speed of the paper production, and the efficiency of the 35 gravity and suction means used to remove water from the wire, and different also for different weights and grades of paper, but, as pointed out, means are provided to secure the steady and uniform flow of a pulp as a thin solution of any 40 desirable consistency from the primary pulp screens to the wire of the paper machine, the points of consistency control being the regulating valve 14 under automatic direction of the thin stock indicator 19, and the hand regulating 45 valve 27, the weight and composition of the paper being controlled by and at the meter 16.

While the paper web is forming on wire 29 most of the water of the paper stock drains through it by gravity to the wire pit 24. Some of the 50 pulp of the paper stock also drains through wire 29, but most of the pulp drainage occurs near breast roll 30 before there has been time for the paper web to form and close the apertures of wire 29. An economy in the process is effected by returning to the stream of paper stock that portion 55 of the drainage which takes place near breast roll 30. To insure the immediate recovery of practically all of the stock lost through wire 29, suitable baffles 31 may be installed in pit 24, thus 60 directing the white water of the higher pulp content to pump 23 and the later drainage over the dam 32 to pit 33, and thence through line 34 to white water storage 35 to which, pulp white water also flows from the thickeners 11 through 65 line 36.

White water from the wire suction boxes (not shown) and or from a suction couch roll 37 may also be flowed to storage 35 through suitable lines (not shown).

From storage 35 white water is impelled by a pump 38 through lines 39 to points in advance of the pulp screens 2 for use in thinning the ground wood pulp as received from the grinders to a consistency suitable for screening.

At times when there may be a deficiency in the amount of screened pulp flowing to vat 4 from screens 2, white water is automatically supplied through line 40 and float valve 41 to vat 4 to compensate for such deficiency. Float valve 41 is located below the crest of dam 10 and under normal operation of the process and apparatus remains closed. It is evident that in case of a complete or a temporary stoppage of the production of ground wood, there is no overflow at dam 10 and no thickened pulp flowing to slush storage 13. In either case the apparatus continues to operate automatically to supply the paper machine until the pulp in slush storage 13 is exhausted, or provided dry pulp is reduced to slush and supplied to storage 13 by the usual breaker means (not shown) the system continues to operate indefinitely.

Customarily, the white water flowing to storage 35 through line 34 is more than sufficient to supply float valve 41, for this water may include clear water used in showers (not shown) to clean the wire 29, but clear water may be supplied to storage 35 through line 42 and float valve 43 to start the process initially, as for instance on a Monday morning after the plant has been shut down over Sunday. However, in the ordinary operation, more white water flows to storage 35 than is required for re-use and the excess is permitted to overflow to recovery filters (not shown) from which point the recovered stock is flowed to the broke storage 44 and the filtered water may be discharged to the mill drains.

Broken paper or broke is reduced to slush pulp by means of a beater 45 supplied with white water for thinning through line 46 from the couch pit 47, the excess from the couch pit overflowing to line 34 and thence to storage 35. Beater 45 discharges to broke storage 44. Pump 48 gradually returns the broke from this storage 44 through line 49 to the ground wood slush storage 13 for re-entrance to the stock circulating system. Stop valves 50 and 51 are for use only when the system is shut down.

Float valves and regulating valves have a tendency to leak in the closed position. As a matter of convenience a small line 52 is provided to care for these leaks and the sample line 20, or to prevent the vat 7 from spilling over when the paper machine is down, but it is desired to leave the indicator 19 and the pump 15 in operation.

The apparatus of Fig. 1 operates automatically to preserve the ground wood pulp as a thin solution from the ground wood screens to the paper machine and the sulphite solution may also be processed in the same manner. Ordinarily from two thirds to three quarters of the number of thickening machines 11 as required in the thick stock process are eliminated as will hereinafter become clearer from an example in which the paper production, the percentage of broke, and all consistencies are fixed at representative values.

In Fig. 2 a method and apparatus is illustrated whereby all of the thickening operation is eliminated. However, the consistency of the pulp solution is necessarily maintained at lower value than that maintained by the apparatus of Fig. 1. This method has a more limited application than that of Fig. 1 because most existing paper machines are unable to accommodate the necessarily lower consistencies maintained and delivered.

In Fig. 2, pulp from the grinders after delivery through line 1 to screens 2 is discharged in its entirety to thin pulp storage 53. From this point it flows to vat 7 through the float valve 8 which

maintains the level in vat 7 at substantially constant elevation. Power driven regulating valve 14 controlled and directed by the thin stock indicator 19 supplied by a continuous sample through line 18 from pump 15, regulates the admission of white water through line 39 to maintain the consistency of the pulp solution at a slightly lower value than that at which the pulp is screened.

Where the method of Fig. 2 is used to regulate the consistency of the ground wood solution, it may be necessary, depending upon the conditions, to use slush sulphite for combining with the ground wood at meter 16 to prevent the consistency of the paper stock from falling too low for delivery to the paper machine and too low to permit the direct return of sufficient white water from pit 24 for economy. The method of Fig. 2 is suitable for new mill construction where the length of wire 29 may be given a sufficient length and the storage 53 made large to compensate for loss of capacity at low consistency.

As a concrete example of the operation of the process as related to Fig. 1, we may assume, a daily paper production of 100 tons per day, (bone dry weight) with 8% broke over and above this production, a required consistency of the paper stock of 0.5%, as it goes to the wire, the use of 18% sulphite in the finished paper, the ground wood to be screened at 0.5% consistency, a portion of the ground wood thickened to 3.09% consistency, a portion of the sulphite thickened to 2.50% consistency, the ground wood white water (using vacuum filters) having a consistency of 0.07%, a supply of 600 gallons per minute of clear water to clean the paper machine wire, and a setting of the thin stock indicator to hold the consistency of the ground wood solution at 0.65%.

Now provided 16 tons per day are returned through line 25 to pump 23, as may be the case, the tons per day going to wire 29 is equal to the daily production of 100 tons, plus 16 tons, plus the 8% broke or 8 tons, and plus an amount flowing through line 34 to storage 35 which is here assumed as 11 tons daily, or to a total of 135 tons per day flowing through head box 28 to wire 29. At 0.5% consistency the rate of flow of paper stock at this point is 4500 gallons per minute. Since 16 tons per day are returned to the wire pit 24, and through line 25 to pump 23, then by subtraction 119 tons per day must come from meter 16, and further, since we have assumed a consistency of 0.65% at meter 16, the 119 tons which flows through this meter daily is a thin solution flowing at the rate of 3050 gallons per minute and a flow of 1450 gallons per minute at a consistency of 0.184% is required in line 25. For simplicity of this explanation or example, we may assume that no stock which is rejected at the paper machine either in the broke or in the white water, is returned to the system in the sulphite, and since the finished paper has a sulphite content of 18%, this pulp is supplied to meter 16 at the rate of 18 tons per day or at the rate of 460 gallons per minute and 0.65% consistency. Subtracting the rate of flow of the sulphite from the rate of flow of the paper stock through line 22, it is found that the rate of flow of the ground wood solution through line 17 is at the rate of 101 tons daily, or 2590 gallons per minute at 0.65% consistency. By the assumptions the ground wood flows through line 6 at 0.5% consistency and through regulating valve 14 at 3.09% consistency and by computation from these values, the flow through line 6 is revealed as 73.4 tons per day or 2444 gallons per

minute and the flow through regulating valve 14 is 27.6 tons per day or 146 gallons per minute. 8 tons of broke per day at 3.09% are returned to the system through line 49 to slush storage 13, thus leaving 19.6 tons per day at 3.09% to be supplied to storage 13 through thickeners 11. From these values, by computation the flow from vat 4 to thickeners 11 is at the rate of 22.28 tons daily or 743 gallons per minute of 0.5% consistency. 19.6 tons daily of this amount are delivered to slush storage 13 through line 12 at the rate of 106 gallons per minute of 3.09% consistency, and the balance or 2.68 tons daily flows through line 36 to storage 35 at the rate of 637 gallons per minute of 0.07% consistency. Thus there is available at pump 38, a total of 4136 gallons per minute for supply to points in advance of screens 2. The tonnage rate through line 3 is equal to the sum of the rates through lines 12 and 6 or 95.68 tons daily which at a consistency of 0.5% amounts to 3197 gallons per minute, leaving an excess of 939 gallons per minute for the recovery filters (not shown) as hereinbefore mentioned.

25 Now comparing the flow through screens 2 with the flow from vat 4 to thickeners 11, it is learned that 23% of the flow through the screens is by-passed to the thickeners, but that 77% of pulp after screening flows directly as a thin solution to meter 16.

Having illustrated and described my invention both in the abstract and with a concrete example of its practical workability, what I claim as new and useful is:

1. The process of making paper comprising, screening a pulp, flowing the main body of the pulp directly to a paper stock meter, thickening some of the pulp to increase the consistency thereof, regulating the rate at which the thickened pulp re-joins the main body of the pulp, supplying other paper making ingredients to said meter, metering each ingredient to form a common stream of paper stock, mixing with said stream a stream of water containing all of the 10 pulp which drains through the paper machine wire near the breast roll and delivering the mixture to the paper machine.

2. The herein described process for making paper consisting in screening a pulp, dividing 15 the screened pulp, flowing one portion directly to a common point for union with other paper making ingredients, extracting white water from the other portion of the pulp, impounding the portion from which white water is extracted, regulating 20 the flow of the impounded pulp to a location of union with the portion flowing to said common point, and metering all ingredients to form a composition for delivery to the paper machine.

3. In a paper making apparatus, the combination of screens for screening a pulp, a meter for metering said pulp, means for moving the screened pulp to said meter, means for diverting some of the screened pulp and extracting some of the water therefrom and means for returning to the 30 screened pulp the portion from which the water was extracted to regulate the consistency of said screened pulp in advance of said meter.

CARLTON H. ALLEN.